



US007604839B2

(12) **United States Patent**  
**McCleskey et al.**

(10) **Patent No.:** **US 7,604,839 B2**  
(45) **Date of Patent:** **Oct. 20, 2009**

(54) **POLYMER-ASSISTED DEPOSITION OF FILMS**

(75) Inventors: **Thomas M. McCleskey**, Los Alamos, NM (US); **Anthony K. Burrell**, Los Alamos, NM (US); **Quanxi Jia**, Los Alamos, NM (US); **Yuan Lin**, Los Alamos, NM (US)

(73) Assignee: **Los Alamos National Security, LLC**, Los Alamos, NM (US)

(\*) Notice: Subject to any disclaimer, the term of this patent is extended or adjusted under 35 U.S.C. 154(b) by 199 days.

(21) Appl. No.: **10/888,868**

(22) Filed: **Jul. 8, 2004**

(65) **Prior Publication Data**

US 2005/0043184 A1 Feb. 24, 2005

**Related U.S. Application Data**

(63) Continuation-in-part of application No. 10/616,479, filed on Jul. 8, 2003, now Pat. No. 7,365,118, which is a continuation-in-part of application No. 09/629,116, filed on Jul. 31, 2000, now Pat. No. 6,589,457.

(51) **Int. Cl.**  
**B05D 3/02** (2006.01)

(52) **U.S. Cl.** ..... 427/226; 427/240; 427/377; 427/385.5; 427/427; 427/427.4; 427/430.1

(58) **Field of Classification Search** ..... 427/226, 427/377, 380, 385.5, 240, 427.1, 427.4, 427, 427/430.1

See application file for complete search history.

(56) **References Cited**

**U.S. PATENT DOCUMENTS**

4,081,576 A \* 3/1978 Hensel et al. ..... 427/393.6

|                 |         |                            |
|-----------------|---------|----------------------------|
| 4,289,816 A     | 9/1981  | Fogelberg et al.           |
| 4,290,918 A *   | 9/1981  | Bayer et al. ..... 502/159 |
| 4,485,094 A     | 11/1984 | Pebler et al.              |
| 4,617,206 A     | 10/1986 | Haisma et al.              |
| 4,931,427 A     | 6/1990  | Chien                      |
| 5,171,735 A     | 12/1992 | Chien                      |
| 5,262,394 A     | 11/1993 | Wu et al.                  |
| 5,314,723 A *   | 5/1994  | Dutta et al. ..... 427/476 |
| 5,318,800 A     | 6/1994  | Gong et al.                |
| 5,382,452 A     | 1/1995  | Bruno et al.               |
| 5,441,767 A     | 8/1995  | DeSaulniers                |
| 5,540,981 A     | 7/1996  | Gallagher et al.           |
| 6,027,766 A     | 2/2000  | Greenberg et al.           |
| 6,255,762 B1    | 7/2001  | Sakamaki et al.            |
| 6,410,934 B1    | 6/2002  | Nayfeh et al.              |
| 6,589,457 B1    | 7/2003  | Li et al.                  |
| 2005/0008777 A1 | 1/2005  | McCleskey et al.           |

**OTHER PUBLICATIONS**

Lang, "Chemical Solution Routes to Single-Crystal Thin Films," *Science*, vol. 273, No. 5277, pp. 903-909, 1996.

Schwartz, "Chemical Solution Deposition of Perovskite Thin Films," *Chemical Materials*, vol. 9, No. 11, pp. 2325-2340, 1997.

\* cited by examiner

*Primary Examiner*—Kirsten C Jolley

(74) *Attorney, Agent, or Firm*—Bruce H. Cottrell; Samuel L. Borkowsky

(57) **ABSTRACT**

A polymer assisted deposition process for deposition of metal oxide films and the like is presented. The process includes solutions of one or more metal precursor and soluble polymers having binding properties for the one or more metal precursor. After a coating operation, the resultant coating is heated at high temperatures to yield metal oxide films and the like. Such films can be epitaxial in structure and can be of optical quality. The process can be organic solvent-free.

**31 Claims, 14 Drawing Sheets**

**Fig. 1**

Fig. 2



Fig. 3





Fig. 4

Fig. 5



Fig. 6



Fig. 7



Fig. 8



Fig. 9



Fig. 10



Fig. 11



Fig. 12



Fig. 13



*Fig. 14*

## 1

## POLYMER-ASSISTED DEPOSITION OF FILMS

This application is a continuation-in-part of U.S. Ser. No. 10/616,479, filed Jul. 8, 2003, by McCleskey et al., which issued as U.S. Pat. No. 7,365,118 on Apr. 29, 2008, which is a continuation-in-part of U.S. Ser. No. 09/629,116, filed Jul. 31, 2000, by Li et al., and issued Jul. 8, 2003 as U.S. Pat. No. 6,589,457.

## STATEMENT REGARDING FEDERAL RIGHTS

This invention was made with government support under Contract No. W-7405-ENG-36 awarded by the U.S. Department of Energy. The government has certain rights in the invention.

## FIELD OF THE INVENTION

The present invention relates to a deposition technique for metal films, metal oxide films, metal nitride films, metal phosphate films, metal boride films, metal fluoride films, metal silicide films, metal chalcogenide films, metal pnictogenide films and the like, and more particularly to the polymer assisted solution deposition of such metal-containing films, especially for deposition of films, metal oxide films, metal nitride films, metal phosphate films, metal boride films, metal fluoride films, metal silicide films, metal chalcogenide films, metal pnictogenide films and the like or epitaxial films, metal oxide films, metal nitride films, metal phosphate films, metal boride films, metal fluoride films, metal silicide films, metal chalcogenide films, metal pnictogenide films and the like.

## BACKGROUND OF THE INVENTION

Metal oxide films are widely used in the electronics industry. Preparation of such metal oxide films has been accomplished by physical vapor deposition techniques such as sputtering, electron beam (e-beam) evaporation, thermal evaporation, molecular beam epitaxy (MBE) and pulsed laser deposition (PLD), by chemical vapor deposition techniques such as plasma-enhanced chemical vapor deposition (PECVD), low-pressure chemical vapor deposition (LPCVD), and metalorganic chemical vapor deposition (MOCVD), and by sol-gel techniques and other chemical solution deposition techniques. Chemical solution deposition techniques have been generally viewed as less capital intensive (see, Lange, "Chemical Solution Routes to Single-Crystal Thin Films", *Science*, vol. 273, pp. 903-909, 1996 and Schwartz, "Chemical Solution Deposition of Perovskite Thin Films", *Chemical Materials*, vol. 9, pp. 2325-2340, 1997). Also, chemical solution techniques are not generally limited to flat surfaces.

Sol-gel techniques are not desirable for many industrial production processes. The sol-gel process uses the high reactivity of organometallic precursors and hydrolyzes these organometallic compounds to make various oligomers. These metal oxo oligomers have suitable viscosity to allow spinning into thin films, which can be fired into ceramic materials at high temperatures. The complication in such a sol-gel process is the uncontrollable polymerization of the metal oxo oligomers because of complex reactive species in the precursor solution. Therefore, the reproducibility of sol-gel processes can be poor which hinders the applications in industrial processes despite the low costs.

## 2

The use of organometallic compounds in chemical solution deposition techniques can be a drawback. As metal salts are typically insoluble in organic solvents, organic moieties have been added to the metal complexes in order to make such metal compounds soluble. This is often undesirable as new reactions and techniques must be developed to incorporate such soluble organic groups onto metal ions. In addition, the resulting organometallic compounds are usually difficult to handle because of their relatively higher reactivity than metal salts.

One problem with the processing of metal salts into ceramic thin films involves the hydrolytic properties of metal ions. Transition metal ions, such as titanium, niobium and tantalum, react with water violently to form metal oxides or metal hydroxides and precipitate out of solution during processing. A more desired methodology to achieve metal oxide films would be a chemical solution having the following properties: clean decomposition to pure ceramics; stable chemical solutions (no gelling) without any reactions before the firing stage; and, the desired viscosity for spin coating, spray coating, or film casting.

U.S. Pat. No. 6,589,457 by Li et al. is directed to deposition of metal oxides from aqueous solutions of water-soluble metal precursors and water-soluble polymers. While none of the examples included a polymer other than polyvinyl alcohol, Li et al. illustrate the continuing efforts in the development of chemical solution deposition processes for production of metal oxide films. The present invention is a continuation of those efforts.

An object of the present invention is to provide a chemical solution deposition method of forming metal oxide films, such a chemical solution deposition method including the deposition of a metal precursor and a soluble polymer where the polymer has binding properties for the metal precursor. In addition to metal oxide films, other films such as metal films, metal nitride films, metal phosphate films, metal boride films, metal silicate films, metal fluoride films, metal chalcogenide films and metal pnictogenide films can be prepared.

Another object of the present invention is to provide a chemical solution deposition method of forming high purity metal oxide films or epitaxial metal oxide films.

Yet another object of the present invention is to provide metal precursor solutions, e.g., metal oxide precursor solutions, having a long shelf-life time in comparison to typical sol-gel solutions.

## SUMMARY OF THE INVENTION

To achieve the foregoing and other objects, and in accordance with the purposes of the present invention, as embodied and broadly described herein, the present invention provides for a process of preparing a uniform highly ordered metal oxide film including applying a homogenous solution, said solution containing a soluble metal precursor and a soluble polymer in a suitable solvent, onto a substrate to form a polymer and metal containing layer thereon, said polymer characterized as having metal binding properties, and, heating said substrate in an oxygen-containing atmosphere at temperatures and for time characterized as sufficient to remove said polymer from said polymer and metal containing layer and form a uniform highly ordered metal oxide film. In one embodiment, the solution further includes a metal-binding ligand or salts thereof.

The present invention further provides a composition of matter including a homogeneous solution of at least two metal precursors and a soluble polymer, the polymer characterized

as having binding properties for the at least two metal precursors, and the at least two metal precursors present in a pre-selected ratio.

The present invention still further provides a composition of matter including a homogenous solution of one or more metal precursors, a soluble polyethyleneimine or polyethyleneimine derivative, and a metal binding ligand or salt thereof, the polyethyleneimine or polyethyleneimine derivative characterized as having binding properties for the one or more metal precursors and the metal selected from alkali metals, alkaline earth metals, main group metals, transition metals other than copper, and lanthanide metals.

The present invention still further provides an article of manufacture including a substrate, and, a uniform conformal coating of a polymer and metal containing layer thereon, said polymer and metal containing layer characterized as having a sufficient metal content whereby heating said substrate in an oxygen-containing atmosphere, a reducing atmosphere or an inert atmosphere, at 250° C. to 1100° C. for a sufficient time removes said polymer from said polymer and metal containing layer to form a uniform highly ordered film, said polymer and metal containing layer further characterized as including a metal binding ligand or salt thereof, and said polymer having binding properties for said metal.

#### BRIEF DESCRIPTION OF THE DRAWINGS

FIG. 1 shows the generic temperature profile of post thermal treatment for epitaxial growth of different oxide films deposited by the polymer assisted deposition technique.

FIG. 2 shows the x-ray diffraction 2θ-scan of a europium oxide (Eu<sub>2</sub>O<sub>3</sub>) film deposited by the process of the present invention on a lanthanum aluminate (LaAlO<sub>3</sub>) substrate. The film is preferentially oriented out of the plane.

FIG. 3 shows the x-ray diffraction φ-scan of (440) Eu<sub>2</sub>O<sub>3</sub> deposited by the process of the present invention on a LaAlO<sub>3</sub> (110) substrate. The film is also oriented in the plane.

FIG. 4 shows a computer generated digital representation of a high-resolution transmission electron microscopy (TEM) of a Eu<sub>2</sub>O<sub>3</sub> film deposited by the process of the present invention on a LaAlO<sub>3</sub> substrate. The interface between the substrate and the film is very sharp. No voids and second phases were detected in the film.

FIG. 5 shows a computer generated digital representation of selected electron diffraction pattern of a Eu<sub>2</sub>O<sub>3</sub> film deposited by the process of the present invention on a LaAlO<sub>3</sub> substrate. The epitaxial nature of the film can be clearly seen from this diffraction pattern.

FIG. 6 shows the x-ray diffraction 2θ-scan of a titanium oxide (TiO<sub>2</sub>) film deposited by the process of the present invention on a R-cut sapphire substrate. The film has a rutile structure and is preferentially oriented out of the plane.

FIG. 7 shows the x-ray diffraction 2θ-scan of a titanium oxide (TiO<sub>2</sub>) film deposited by the process of present invention on a lanthanum aluminate (LaAlO<sub>3</sub>) substrate. The film has an anatase structure and is preferentially oriented out of the plane.

FIG. 8 shows the x-ray diffraction φ-scan of anatase (101) TiO<sub>2</sub> and (101) LaAlO<sub>3</sub> substrate. The anatase phase is formed by the process of present invention. The film is oriented in the plane.

FIG. 9 shows the x-ray diffraction 2θ-scan of a YBa<sub>2</sub>Cu<sub>3</sub>O<sub>7-x</sub> (YBCO) film deposited by the process of present invention on a LaAlO<sub>3</sub> substrate. The film is highly c-axis oriented.

FIG. 10 shows the x-ray diffraction φ-scan of (102) YBCO and (101) LaAlO<sub>3</sub> substrate. The film was deposited by the process of present invention. The YBCO is epitaxial as seen by FIGS. 9 and 10.

FIG. 11 shows the x-ray diffraction 2θ-scan of a BaTiO<sub>3</sub> film deposited by the process of present invention on a LaAlO<sub>3</sub> substrate. The film is highly oriented out of the plane.

FIG. 12 shows the x-ray diffraction φ-scan of (101) BaTiO<sub>3</sub> and (101) LaAlO<sub>3</sub> substrate. The film was deposited by the process of present invention. The BaTiO<sub>3</sub> is epitaxial as seen by FIGS. 11 and 12.

FIG. 13 shows the x-ray diffraction 2θ-scan of a SrTiO<sub>3</sub> film deposited by the process of present invention on a LaAlO<sub>3</sub> substrate. The film is highly oriented out of the plane.

FIG. 14 shows the x-ray diffraction φ-scan of (202) SrTiO<sub>3</sub> and (202) LaAlO<sub>3</sub> substrate. The film was deposited by the process of present invention. The SrTiO<sub>3</sub> is epitaxial as seen by FIGS. 13 and 14.

#### DETAILED DESCRIPTION

The present invention is concerned with a process for preparing metal-containing films such as metal films, metal oxide films, metal nitride films and the like, from solutions, optionally in an organic solvent-free process. The metal oxide films can be prepared with an epitaxial structure. The elimination of organic solvents from chemical solution deposition techniques can be preferred in some instances. Additionally, it has been found that the metal-containing films made in accordance with the present invention can be formed crack-free. This is in contrast to the cracking that sometimes resulted in various prior techniques.

The process of the present invention uses a soluble polymer to assist in the deposition of the desired metal oxide. Thus, the process can be referred to as a polymer assisted deposition process. Inclusion of a soluble polymer with a single metal precursor or multiple metal precursors promotes better distribution of the materials during the deposition. The polymer can be removed subsequently by heating at sufficiently high temperatures to eliminate the polymer and leave a metal oxide film. The resultant metal oxide film can be prepared with orientation, i.e., the film can be prepared with an epitaxial structure. By using a soluble polymer in conjunction with one or more metal precursors, single or mixed compound/complex metal oxide films can be prepared. In one embodiment, the overall process can be an aqueous process that can be organic solvent free. Depending upon the selection of precursor and atmosphere during heating, other films such as metal films, metal nitride films, metal phosphate films, metal boride films, metal silicate films, metal fluoride films, metal chalcogenide films and metal pnictogenide films can be prepared.

The heating of the polymer and metal layer is generally carried out under an inert atmosphere, a reducing atmosphere, or an oxygen-containing atmosphere. Of example, in the case where it is desired to reduce a metal precursor to obtain a metal film, the reducing atmosphere can include, e.g., hydrogen, ammonia, formaldehyde, carbon monoxide, formic acid or other reducing agents well known to those skilled in the art. A reducing atmosphere can also be used in the preparation of metal nitride, metal boride, metal chalcogenide, and metal pnictogenide films. Suitable inert atmospheres can generally be argon, nitrogen and the like. For preparation of metal oxides, an oxygen-containing atmosphere will generally be used.

While a metal oxide film can be prepared with an highly ordered structure, e.g., an epitaxial structure, by the process of the present invention, it may also be prepared with an

amorphous structure, a nanocrystalline structure or a polycrystalline structure by suitable treatment after deposition of the polymer and metal containing layer upon a substrate or by suitable selection of the substrate. By "highly ordered" is meant ordering with a preferred orientation as can be seen in XRD measurements. Such amorphous or polycrystalline structures may be preferred for some applications.

The metal-containing films (the metal, the oxide, the nitride and the like) of the present invention are uniform films, i.e., they are continuous films covering the target substrate. They can also be readily formed as conformal films upon non-planar substrates or surfaces.

The soluble polymer used in the present process has binding properties for the metal precursors used to form the metal oxide film and can be, e.g., polyethyleneimine (PEI), a substituted PEI or PEI derivative such as a carboxylated-polyethyleneimine (PEIC), a phosphorylated-polyethyleneimine (PEIP), a sulfonated-polyethyleneimine (PEIS), an acylated-polyethyleneimine, hydroxylated water-soluble polyethyleneimines and the like or a polymer such as polyacrylic acid, polypyrrolidone, and poly(ethylene-maleic acid). PEI or substituted PEIs such as PEIC are generally the preferred polymers. Substituted or PEI derivatives are post modified after formation of the base polymer. Typically, the molecular weight of such polymers is greater than about 30,000. By "binding" it is meant that the polymer and the metal are bound through any of various mechanisms such as electrostatic attraction, hydrogen bonding, covalent bonding and the like.

In order to have good processing characteristics, a precursor solution for metal oxide films must have a suitable viscosity. In the present invention, polymer plays dual functions. In other words, a polymer is also used to assist the viscosity desired for metal oxide film processing.

The solutions used in depositing the polymer and metal to the substrates are homogeneous solutions. By "homogeneous" is meant that the solutions are not dispersions or suspensions, but are actual solutions of the polymer, metal complexes and any metal binding ligands.

The criteria on the choice of polymers are that they be soluble, undergo a clean decomposition upon heating at high temperatures, e.g., temperatures over about 250° C., and are compatible with the metal compounds. PEI decomposes completely and cleanly above 250° C. and leaves no residual carbon in the film. This feature makes PEI and derivatives thereof especially preferred polymers in the practice of the present invention.

By aiding in the desired viscosity, such polymers can allow processing of the metal oxide precursor solution into desired configurations such as films. The desired viscosity can be achieved through controlling the solution concentration of the soluble polymers and by controlling the molecular weight of the polymer. For high quality homogeneous films, polymer concentrations and the polymer ratio to metal components should be maintained at a proper balance. The rheology of the metal oxide precursor solution can also be important for the morphology and quality of the final metal oxide films. In order to form smooth films, the polymer solution must have suitable rheological properties so that any spin-coated film has no undesired patterns associated with polymer rheological properties.

The polymer further functions as binding agent to the metals within the precursor solution in assisting the formation of an intermediate deposited polymer-metal composite film and ultimately a metal oxide film. This requires that the polymer should also have suitable interactions to metal ions such that no phase separation occurs during the deposition processes. Thereafter, the deposited polymer-metal composite films are

heated at high temperatures (calcined), e.g., at temperatures above about 250° C. to obtain the final metal oxide films. Thus, the soluble polymer selection should also have suitable decomposition characteristics, e.g., a clean decomposition under such calcination conditions, so that the final metal oxide film can be free of side products.

The general approach of the present invention can be applied to main group metals, transition group metals and lanthanide metals in forming resultant metal oxides, metal nitrides, metal phosphates, metal borides, metal silicides, metal fluorides, metal chalcogenides, metal pnictogenides or metals. Among the main group metals are included aluminum, gallium, germanium, silicon, indium, tin, antimony, lead, and bismuth.

Among the transition metals are included titanium, vanadium, chromium, manganese, iron, cobalt, nickel, copper, zinc, yttrium, zirconium, niobium, palladium, platinum, molybdenum, ruthenium, rhodium, cadmium, hafnium, tantalum, tungsten, rhenium, osmium, and iridium.

Among the lanthanide metals are included lanthanum, cerium, praseodymium, neodymium, samarium, europium, gadolinium, terbium, dysprosium, holmium, erbium, thulium, ytterbium and lutetium.

Other metals such as alkaline earth metals including calcium, strontium and barium can generally be one metal component in mixed metal oxides such as calcium titanate, calcium ruthenate, barium titanate, barium ruthenate, strontium titanate, strontium ruthenate, yttrium barium copper oxide. Simple oxides such as MgO and SrO can be also prepared by this method.

Still other metals such as alkali metals including sodium, lithium and potassium may generally be one metal component in mixed metal oxides such as lithium tantalate (LiTaO<sub>3</sub>), lithium niobate (LiNbO<sub>3</sub>), Fe- or Ti-doped lithium niobate, potassium barium niobate (KBa<sub>2</sub>Nb<sub>5</sub>O<sub>15</sub>), potassium lithium niobate (K<sub>3</sub>Li<sub>2</sub>Nb<sub>5</sub>O<sub>15</sub>), potassium sodium tantalate ((K<sub>1-x</sub>Na<sub>x</sub>)TaO<sub>3</sub>), K<sub>3</sub>Li<sub>2</sub>(Ta<sub>x</sub>Nb<sub>1-x</sub>)O<sub>15</sub> and the like.

The present invention may also employ fluoride complexes as precursors in the process of the present invention. For example, a gallium hexafluoride anion (GaF<sub>6</sub><sup>3-</sup>) can be formed by the addition of gallium nitrate and ammonium bifluoride and can be used as the metal precursor.

The metal oxide films prepared by the present process can include a metal oxide with a single metal, can be a metal oxide with two metals or three metals or may be a metal oxide including four or more metals. Among the metal oxides that can be prepared by the present process are included titanium oxide, magnesium oxide, zinc oxide, ruthenium oxide and the like. Among the mixed metal oxides that can be prepared by the present process are included barium titanium oxide (barium titanate), strontium titanium oxide (strontium titanate), barium strontium titanium oxide (barium strontium titanate), strontium ruthenium oxide (strontium ruthenate), lanthanum-strontium manganese oxide, yttrium-barium-copper oxide (YBa<sub>2</sub>Cu<sub>3</sub>O<sub>7</sub>) and the like. The metal oxide films prepared by the present process can be insulating, resistive, conductive, ferroelectric, ferromagnetic, piezoelectric, and even superconductive depending upon the chemical compositions and microstructures.

Metal nitride films that can be prepared by the present process can include a metal nitride with a single metal, can be a metal nitride with two metals or three metals or may be a metal nitride including four or more metals. Among the metal nitrides that can be prepared by the present process are included titanium nitride, gallium nitride and tantalum nitride and the like. Among the mixed metal nitrides that can be prepared by the present process are included tantalum nio-

bium nitride and the like. The metal nitride films prepared by the present process can be serve as wide bandgap semiconductors and as hardening materials and can be insulating, resistive, conductive, ferroelectric, ferromagnetic, and piezoelectric, depending upon the chemical compositions and microstructures. The preparation of metal nitride films can be accomplished by depositing a polymer and metal containing layer upon a suitable substrate as with a metal oxide, but the heating can then be conducted under an ammonia-containing atmosphere, a reducing atmosphere or an inert atmosphere to yield the desired nitride materials.

Metal phosphate films that can be prepared by the present process can include a metal phosphate with a single metal, can be a metal phosphate with two metals or three metals or may be a metal phosphate including four or more metals. Among the metal phosphates that can be prepared by the present process are included zirconium phosphate, molybdenum phosphate and the like. Among the mixed metal phosphates that can be prepared by the present process are included tungsten molybdenum phosphate and the like. The metal phosphate films prepared by the present process can be insulating, resistive, conductive, ferroelectric, ferromagnetic, and piezoelectric and may be useful as catalytic materials, depending upon the chemical compositions and microstructures. The preparation of metal phosphate films can be accomplished by depositing a polymer and metal containing layer upon a suitable substrate as with a metal oxide, but the heating can then be conducted under an inert atmosphere to yield the desired phosphate materials. Suitable phosphate precursors for inclusion in a homogenous solution of the present invention can include phosphoric acid or may include phosphate esters and phosphines and the like.

Metal boride films that can be prepared by the present process can include a metal boride with a single metal, can be a metal boride with two metals or three metals or may be a metal boride including four or more metals. Among the metal borides that can be prepared by the present process are included cobalt boride, magnesium boride and the like. Among the mixed metal borides that can be prepared by the present process are included cobalt magnesium boride and the like. The metal boride films prepared by the present process can be insulating, resistive, conductive, ferroelectric, ferromagnetic, and piezoelectric and may be superconductive as well, depending upon the chemical compositions and microstructures. The preparation of metal boride films can be accomplished by depositing a polymer and metal containing layer upon a suitable substrate as with a metal oxide, but the heating can then be conducted under an inert atmosphere or a reducing atmosphere to yield the desired boride materials. Suitable boride precursors for inclusion in a homogenous solution of the present invention may include borohydrides, alkyl borates such as tetraphenyl borate, and the like.

In addition to metal nitride films, similar or other metal pnictogenides such as metal arsenides (e.g., gallium arsenide) or metal phosphides (e.g., gallium phosphide) may be prepared by the present process. The preparation of metal pnictogenide films can be accomplished by depositing a polymer and metal containing layer upon a suitable substrate as with a metal oxide, but the heating can then be conducted under an inert atmosphere to yield the desired pnictogenide materials. The metal pnictogenide films prepared by the present process can be insulating, resistive, conductive, ferroelectric, ferromagnetic, and piezoelectric, depending upon the chemical compositions and microstructures. Suitable pnictogenide precursors for inclusion in a homogenous solution of the present invention can include arsenide trichloride or may include other tris(trimethylsilyl)X where X is P, As or Sb.

In addition to metal oxide films, similar or other metal chalcogenide films that can be prepared by the present process can include a metal chalcogenide with a single metal (e.g., zinc telluride and the like), can be a metal chalcogenide with two metals or three metals (e.g., zinc cadmium telluride and the like) or may be a metal chalcogenide including four or more metals. The metal chalcogenide films prepared by the present process can be insulating, resistive, conductive, ferroelectric, ferromagnetic, and piezoelectric, depending upon the chemical compositions and microstructures. The preparation of metal chalcogenide films can be accomplished by depositing a polymer and metal containing layer upon a suitable substrate as with a metal oxide, but the heating can then be conducted under an inert atmosphere or reducing atmosphere to yield the desired chalcogenide materials. The chalcogenides can include selenides, tellurides and the like. Suitable chalcogenide precursors for inclusion in a homogenous solution of the present invention may include dialkyl selenide, tellurium dichloride and the like.

Metal oxide clusters can be employed as anions bound to a polymer in the present invention. In this manner, metal silicides may be prepared by the present process using a sodium silicon water glass (e.g., a 50/50 weight % solution of Na and Si containing negatively charged silicate oligomers). Other metal oxide clusters such as sodium orthovanadate or sodium tungstate can also be used.

In one aspect of the present invention, composites can be prepared including the various metal-containing films as described with various additional additives to provide tailoring of the material properties. Among the additives can be nanoparticles, especially nanoparticles of various metals such as transition metals, lanthanide metals or main group metals, nanoparticles of various metal oxides including one or more metal such as a transition metal, a lanthanide metal or a main group metal, nanoparticles of various metal nitrides including one or more metal such as a transition metal, a lanthanide metal or a main group metal, nanoparticles of various metal carbides including one or more metal such as a transition metal, a lanthanide metal or a main group metal, nanoparticles of various metal chalcogenides including one or more metal such as a transition metal, a lanthanide metal or a main group metal, nanoparticles of various metal pnictogenides including one or more metal such as a transition metal, a lanthanide metal or a main group metal, nanoparticles of various metal borides including one or more metal such as a transition metal, a lanthanide metal or a main group metal, or nanoparticles of various metal silicides including one or more metal such as a transition metal, a lanthanide metal or a main group metal. Examples of such nanoparticles can include titanium dioxide, strontium oxide, erbium oxide and the like, such nanoparticles suitable for modifying the electronic properties of metal oxide films of a different material.

Other additives may include silicon beads, which may provide void properties to the various metal containing films in accordance with the present invention. Additionally, various dendrimer systems such as PAMAM-4 dendrimer (available from Aldrich Chemical Co.) and the like may be added and may provide a dopant to the various metal containing films in accordance with the present invention. Also, various quantum dot materials, e.g., cadmium selenide dots having a coating of zinc sulfide, such quantum dot materials being well known to those skilled in the art, may be added to the various metal containing films in accordance with the present invention.

The composition, e.g., solution, used for the deposition includes the soluble polymer and the metal precursors. In addition, other metals can be included through addition of

appropriate metal salts. For example, barium can be added through a barium salt such as barium acetate. Other suitable metal salts may include metal nitrates, metal oxalates, metal acrylates, and metal coordination complexes.

The solvent for dissolution of the soluble polymer can be, e.g., water, lower alcohols such as methanol, ethanol, propanol and the like, acetone, propylene carbonate, tetrahydrofuran, acetonitrile, acetic acids and mixtures thereof such as water and ethanol and the like. As the soluble polymer used in the present invention includes binding properties for the metals or metal precursors used in formation of the metal oxide films, the polymer can help provide the necessary solubility to the respective metals, e.g., metal precursors. In some instances, the metal can initially be in a metal complex such as a complex of the respective metal with a metal binding ligand or salt thereof such as ethylenediaminetetraacetic acid (EDTA) or salts thereof such as dipotassium ethylenediaminetetraacetic acid. EDTA-metal complexes are generally soluble within solutions including a soluble polymer with binding properties for the metal precursors such as PEI and the like.

Among suitable metal binding ligands besides EDTA and salts thereof can be included other carboxylic acid ligands such as ethylenediaminediacetic acid (EDDA), trans-1,2-diamino-cyclohexan-N,N,N',N'-tetraacetic acid (CDTA), ethyleneglycol-O,O'-bis-(2-aminoethyl)-N,N,N',N'-tetraacetic acid (EGTA), diethylenetriamine-pentaacetic acid (DTPA), N-(2-hydroxyethyl)-ethylenediamine-N,N',N'-triacetic acid (HEDTA), nitrilotriacetic acid (NTA), triethylenetetramine-N, N,N',N",N",N"-hexaacetic acid (TTHA) and the like, poly-pyridyl ligands such as terpyridine, 2,2'-bipyridine, 1,10-phenanthroline and the like, beta-diketone (acetylacetone) ligands such as 2,4-propanedione and derivatives thereof, catecholate and aryl oxide or alkyl oxide ligands, macrocyclic ligands such as cyclam, cyclen, triazacyclononane and derivatives thereof, or other simple ligands such as aquo ( $H_2O$ ) and amines ( $NH_3$ ), i.e.,  $Co(NH_3)_6^{2+}$ . Schiff-base ligands such as trimethylenediaminetetramethylglyoximate ligand or the salen type ligands may also be used.

The starting solution is typically maintained at ambient temperatures from about 15° C. to about 30° C., more usually from about 20° C. to about 25° C. Within those temperature ranges, the materials added to the solution are soluble. In preparation of solutions used in the present process, the solutions using a polyethyleneimine as the metal binding polymer can be filtered prior to use to remove any non-soluble components. One exemplary process in the preparation of the solutions involves filtering the precursor solution through an Amicon ultrafiltration unit containing a PM 10 ultrafiltration membrane. Such a filter is designed to pass materials having a molecular weight of less than about 10,000 g/mol (e.g., unbound metal, smaller polymer fragments and the like) while retaining the desired materials of a larger size. Ultrafiltration allows for removal of any unwanted salts such as cations, anions or other impurities.

The metal ratio can be controlled through appropriate addition of metal precursors to the solvent used in the deposition. Such solutions can generally have a shelf life of more than a year.

In one embodiment of the present invention, the starting solution can be deposited on a desired substrate, e.g., by spray coating, dip coating, spin coating, ink jet printing and the like. After deposition of the starting solution on a substrate, the deposited coating must be calcined or heated at high temperatures of from about 250° C. to about 1300° C., preferably from about 400° C. to about 1200° C. for a period of time sufficient to remove the polymer and to form only the metal

oxide film. FIG. 1 shows a general temperature profile of the thermal treatment for growth of metal oxide films deposited by the process of this invention. Heating times may be varied and may be longer depending upon the thickness of the deposited film.

Optionally, the deposited coating can be initially dried by heating to temperatures of from about 50° C. to about 150° C. for from about 15 minutes to several hours, preferably for less than one hour. The deposited polymer-metal oxide film undergoes removal of a percentage of volatile species during such an initial drying stage.

The resultant metal oxide films from the present process have been optical quality films in that they are highly smooth films with a mirror-like appearance. Many of the films have been found to be epitaxial in structure.

The present invention enables the processing of metal oxide films with convenience and flexibility required in industrial fabrication. This process involves making metal oxide films from solutions—optionally in an organic solvent-free process. Barium titanate ( $BaTiO_3$ ) and strontium titanate ( $SrTiO_3$ ) films have been prepared using polymer-assisted aqueous deposition (PAD) techniques. X-ray diffraction measurement indicates that the barium titanate and strontium titanate films on  $LaAlO_3$  are preferentially oriented along the (100). They are also epitaxial as confirmed from x-ray  $\phi$ -scans of the (101) diffraction of the films and transmission electron microscopy.

The polymer is used to bind metals and metal precursors. This allows the removal of any unwanted anions or cations by filtration, e.g., through an Amicon ultrafiltration unit, and brings multiple metals together in a homogeneous manner at a molecular level. This also prevents selective precipitation of unwanted metal oxide phases as a portion of the water can be removed and the metals concentrated within the remaining solution. Even at the extreme of just polymer and metal, the dried solution (a gel) includes only well dispersed metal atoms bound to the polymer. The present invention has extended the potential of controlling relative metal concentrations at the molecular level for mixed metal oxides such as superconductors ( $YBa_2Cu_3O_{7-x}$ ). This can be done in one of three ways.

In a first manner, a single polymer (such as carboxylated polyethyleneimine) can be added to a solution containing simple salts (such as nitrate) of two or more metals in the correct ratio. If the binding constant is high for both metals then they will remain in the correct ratio during filtration and concentration of the polymer.

In a second manner, the metals can be bound individually to one or more polymers and concentrated. The resulting solution can be examined by ICP to determine metal content and then mixed appropriately prior to spin coating. Different polymers and different solvents can be used for different metals in this system.

In a third manner, metal complexes such as a metal-EDTA complex can be prepared and mixed in the desired ratios. These complexes can then be bound to a polymer (such as polyethyleneimine) and concentrated.

The present invention is more particularly described in the following examples that are intended as illustrative only, since numerous modifications and variations will be apparent to those skilled in the art.

Examples A-DD describe the preparation of solutions used in the deposition and formation of the metal oxide films, metal films or other metal containing films. Examples 1-16 describe the deposition of such metal oxide films, metal films or other metal containing films using such solutions. Polyethyleneimine was obtained from BASF as a water free,

11

branched, polymer with an average MW of 50,000. Water was deionized via reverse osmosis (having a resistivity >16 Ohms).

## EXAMPLE A

A solution including zinc chloride and polyethyleneimine was prepared as follows. An amount of 4.4 grams of polyethyleneimine was dissolved in 40 mL of water and the pH was adjusted to pH 6 with addition of 10% HCl. To this solution was added 2.2 grams of  $ZnCl_2$  and the solution was stirred. After stirring the solution was placed in an Amicon ultrafiltration unit containing a PM 10 ultrafiltration membrane designed to pass materials having a molecular weight <10,000 g/mol. The solution was diluted to 200 mL and then concentrated to 45 mL in volume. Inductively coupled plasma-atomic emission spectroscopy showed that the final solution had 21.1 mg/mL of Zn.

## EXAMPLE B

A solution including zinc nitrate and polyethyleneimine was prepared as follows. An amount of 2.0 grams of polyethyleneimine was dissolved in 40 mL of water and the pH was adjusted to pH 6 with addition of 10% HCl. To this solution was added 2.5 grams of zinc nitrate hexahydrate and the solution was stirred. After stirring the solution was placed in an Amicon ultrafiltration unit containing a PM 10 ultrafiltration membrane designed to pass materials having a molecular weight <10,000 g/mol. The solution was diluted to 200 mL and then concentrated to 20 mL in volume. Inductively coupled plasma-atomic emission spectroscopy showed that the final solution had 24.2 mg/mL of Zn.

## EXAMPLE C

A solution including zinc chloride, dipotassium ethylenediaminetetraaceticacid (EDTA K<sub>2</sub>) and polyethyleneimine was prepared as follows. An amount of 2.0 grams of dipotassium ethylenediaminetetraaceticacid was dissolved in 30 mL of water. To this solution was added 0.75 grams of zinc chloride and the solution was stirred. After stirring, 2 grams of polyethyleneimine were added and the pH was adjusted to 9 with addition of 10% HCl. The solution was placed in an Amicon ultrafiltration unit containing a PM 10 ultrafiltration membrane designed to pass materials having a molecular weight <10,000 g/mol. The solution was diluted to 200 mL and then concentrated to 20 mL in volume. Inductively coupled plasma-atomic emission spectroscopy showed that the final solution had 24.2 mg/mL of Zn.

## EXAMPLE D

A solution including copper nitrate and polyethyleneimine was prepared as follows. One gram of polyethyleneimine (from BASF) was placed in a 50 mL Falcon tube and dissolved in 25 mL of water. Then, 0.85 grams of copper nitrate trihydrate were added. After stirring the solution was placed in an Amicon ultrafiltration unit containing a PM 10 ultrafiltration membrane designed to pass materials having a molecular weight <10,000 g/mol. The solution was diluted to 200 mL and then concentrated to 10 mL in volume. Inductively coupled plasma-atomic emission spectroscopy showed that the final solution had 15.2 mg/mL of Cu.

## EXAMPLE E

A solution including copper nitrate, ethylenediaminetetraaceticacid and polyethyleneimine was prepared as follows.

12

One gram of ethylenediaminetetraaceticacid was placed in a 50 mL Falcon tube and 25 mL of water were added. The ethylenediaminetetraaceticacid does not dissolve at this stage. One gram of polyethyleneimine (from BASF) was added to the solution and the solution was agitated until the ethylenediaminetetraaceticacid and the polyethyleneimine were in solution. Then 0.85 grams of copper nitrate trihydrate were added. After stirring the solution was placed in an Amicon ultrafiltration unit containing a PM 10 ultrafiltration membrane designed to pass materials having a molecular weight <10,000 g/mol. The solution was diluted to 200 mL and then concentrated to 10 mL in volume. Inductively coupled plasma-atomic emission spectroscopy showed that the final solution had 15.2 mg/mL of Cu.

## EXAMPLE F

A solution including yttrium nitrate, ethylenediaminetetraaceticacid and polyethyleneimine was prepared as follows. One gram of ethylenediaminetetraaceticacid was placed in a 50 mL Falcon tube and 25 mL of water were added. The ethylenediaminetetraaceticacid does not dissolve at this stage. One gram of polyethyleneimine (from BASF) was added to the solution and the solution was agitated until the ethylenediaminetetraaceticacid and the polyethyleneimine were in solution. Then 1.36 grams of yttrium nitrate hexahydrate were added. After stirring the solution was placed in an Amicon ultrafiltration unit containing a PM 10 ultrafiltration membrane designed to pass materials having a molecular weight <10,000 g/mol. The solution was diluted to 200 mL and then concentrated to 10 mL in volume. Inductively coupled plasma-atomic emission spectroscopy showed that the final solution had 15.3 mg/mL of Y.

## EXAMPLE G

A solution including barium nitrate, ethylenediaminetetraaceticacid and polyethyleneimine was prepared as follows. One gram of ethylenediaminetetraaceticacid was placed in a 50 mL Falcon tube and 25 mL of water were added. The ethylenediaminetetraaceticacid does not dissolve at this stage. One gram of polyethyleneimine (from BASF) was added to the solution and the solution was agitated until the ethylenediaminetetraaceticacid and the polyethyleneimine were in solution. Then 0.90 grams of barium nitrate were added. After stirring the solution was placed in an Amicon ultrafiltration unit containing a PM 10 ultrafiltration membrane designed to pass materials having a molecular weight <10,000 g/mol. The solution was diluted to 200 mL and then concentrated to 10 mL in volume. Inductively coupled plasma-atomic emission spectroscopy showed that the final solution had 29.5 mg/mL of Ba.

## EXAMPLE H

A solution including barium hydroxide, ethylenediaminetetraaceticacid and polyethyleneimine was prepared as follows. An amount of 1.4 grams of ethylenediaminetetraaceticacid was placed in a 50 mL Falcon tube and 25 mL of water were added. The ethylenediaminetetraaceticacid does not dissolve at this stage. 1.4 grams of polyethyleneimine (from BASF) were added to the solution and the solution was agitated until the ethylenediaminetetraaceticacid and the polyethyleneimine were in solution. Then 1.50 grams of water insoluble barium hydroxide octahydrate were added. After stirring the solution was placed in an Amicon ultrafiltration unit containing a PM 10 ultrafiltration membrane designed to

13

pass materials having a molecular weight <10,000 g/mol. The solution was diluted to 200 mL and then concentrated to 14 mL in volume. Inductively coupled plasma-atomic emission spectroscopy showed that the final solution had 28.8 mg/mL of Ba.

## EXAMPLE I

A solution including titanium and peroxide and PEIC was prepared as follows. An amount of 1.0 gram of PEIC (PEI with  $\frac{1}{2}$  of the amine sites functionalized into carboxylates) was dissolved in 30 mL of water. A solution of soluble titanium was prepared by placing 2.5 grams of 30% peroxide into 30 mL of water and then slowly adding 2.5 grams of titanium tetrachloride. Small aliquots of 1 mL of the titanium solution were then added to the PEIC solution and the pH was monitored as the pH increased above 3.5 aliquots of 10% NaOH were added to lower the pH to 7.5. This process was repeated until addition of the titanium solution resulted in precipitate that would not dissolve. The solution was then filtered and was placed in an Amicon ultrafiltration unit containing a PM 10 ultrafiltration membrane designed to pass materials having a molecular weight <10,000 g/mol. The solution was diluted to 200 mL and then concentrated to 10 mL in volume. Inductively coupled plasma-atomic emission spectroscopy showed that the final solution had 4.6 mg/mL of Ti.

## EXAMPLE J

A solution including strontium nitrate and ethylenediaminetetraaceticacid and polyethyleneimine was prepared as follows. An amount of 1.7 grams of ethylenediaminetetraaceticacid was placed in a 50 mL Falcon tube and 25 mL of water were added. The ethylenediaminetetraaceticacid does not dissolve at this stage. 1.7 grams of polyethyleneimine (from BASF) were added to the solution and the solution was agitated until the ethylenediaminetetraaceticacid and the polyethyleneimine were in solution. Then 1.22 grams of strontium nitrate were added. After stirring the solution was placed in an Amicon ultrafiltration unit containing a PM 10 ultrafiltration membrane designed to pass materials having a molecular weight <10,000 g/mol. The solution was diluted to 200 mL and then concentrated to 17 mL in volume. Inductively coupled plasma-atomic emission spectroscopy showed that the final solution had 16.0 mg/mL of Sr.

## EXAMPLE K

A solution including cadmium nitrate and ethylenediaminetetraaceticacid and polyethyleneimine was prepared as follows. An amount of 2.0 grams of polyethyleneimine was dissolved in 40 mL of water and the pH was adjusted to pH 6 with addition of 10% HCl. 2.5 grams of cadmium nitrate tetrahydrate were added and the solution was stirred. After stirring the solution was placed in an Amicon ultrafiltration unit containing a PM 10 ultrafiltration membrane designed to pass materials having a molecular weight <10,000 g/mol. The solution was diluted to 200 mL and then concentrated to 20 mL in volume. Inductively coupled plasma-atomic emission spectroscopy showed that the final solution had 37.6 mg/mL of Cd.

## EXAMPLE L

A solution including indium nitrate, ethylenediaminetetraaceticacid and polyethyleneimine was prepared as follows. One gram of ethylenediaminetetraaceticacid was placed in a

14

50 mL Falcon tube and 25 mL of water were added. The ethylenediaminetetraaceticacid does not dissolve at this stage. One gram of polyethyleneimine was added to the solution and the solution was agitated until the ethylenediaminetetraaceticacid and the polyethyleneimine were in solution. Then 1.00 grams of indium nitrate were added. After stirring the solution was placed in an Amicon ultrafiltration unit containing a PM 10 ultrafiltration membrane designed to pass materials having a molecular weight <10,000 g/mol. The solution was diluted to 200 mL and then concentrated to 10 mL in volume. Inductively coupled plasma-atomic emission spectroscopy showed that the final solution had 14.2 mg/mL of In.

## EXAMPLE M

A solution including tin (II) chloride and PEIC was prepared as follows. An amount of 1.0 gram of PEIC (PEI with  $\frac{1}{2}$  of the amine sites functionalized into carboxylates) was dissolved in 30 mL of water. To this solution was added 0.65 grams of tin(II) chloride. After stirring the solution was placed in an Amicon ultrafiltration unit containing a PM 10 ultrafiltration membrane designed to pass materials having a molecular weight <10,000 g/mol. The solution was diluted to 200 mL and then concentrated to 10 mL in volume. Inductively coupled plasma-atomic emission spectroscopy showed that the final solution had 15.5 mg/mL of Sn.

## EXAMPLE N

A solution including gallium chloride and polyethyleneimine in ethanol was prepared as follows. An amount of 5 grams of polyethyleneimine were dissolved in 95 grams of ethanol. The solution was dried over molecular sieves for two days and then filtered through a 0.49 micron filter. About 20 mL of the solution were placed in a 50 mL Falcon tube and 0.6 grams of gallium chloride were added in an inert atmosphere. A precipitate appears and then dissolves into solution. This solution was placed in an Amicon ultrafiltration unit containing a YM 10 ultrafiltration membrane designed to pass materials having a molecular weight <10,000 g/mol. The solution was diluted to 200 mL with absolute ethanol and then concentrated to 10 mL in volume. After filtration, the viscosity of the solution was further increased by removing a small amount of solvent by rotary evaporation under reduced pressure. Inductively coupled plasma-atomic emission spectroscopy showed that the final solution had 14.3 mg/mL of Ga.

## EXAMPLE O

A solution including indium and tin was prepared as follows. An amount of 5.0 grams of the final solution from example L was mixed with 5.0 grams of the final solution from example M to yield a solution equal molar in In and Sn.

## EXAMPLE P

A solution including barium and titanium was prepared as follows. An amount of 5.0 grams of the final solution from example I was mixed with 2.21 grams of the final solution from example G to yield a solution equal molar in Ti and Ba.

## EXAMPLE Q

A solution including strontium and titanium was prepared as follows. An amount of 5.0 grams of the final solution from

## 15

example I was mixed with 2.59 grams of the final solution from example J to yield a solution equal molar in Ti and Sr.

## EXAMPLE R

A solution including yttrium barium and copper was prepared as follows. An amount of 5.0 grams of the final solution from example F was mixed with 8.0 grams of the final solution from example G and 10.0 grams of the final solution from example E to yield a solution with molar ratios of 1:2:3 for Y:Ba:Cu.

## EXAMPLE S

A solution including yttrium barium and copper was prepared as follows. A  $\text{YBa}_2\text{Cu}_3$  solution was also prepared by addition of 2.0 grams polyethylenimine and 2.0 grams ethylenediaminetetraacetic acid to a solution of the metal nitrates having an a ratio of Y:Ba:Cu equal to 1:2:3 (0.47 grams yttrium nitrate hexahydrate, 0.64 grams barium nitrate and 0.89 grams copper nitrate trihydrate). The solution was then concentrated by rotary evaporation under reduced pressure. This solution can be used for coating without filtration since nitrates decompose readily to gases. Alternatively hydroxide and other salts that thermally degrade can also be used.

## EXAMPLE T

A solution including cadmium and zinc and polyethylenimine was prepared as follows. An amount of 2.0 grams of polyethylenimine was dissolved in 40 mL of water and the pH was adjusted to pH 6 with addition of 10% HCl. To this solution was added 1.6 grams of zinc nitrate hydrate and 0.4 grams of cadmium nitrate tetrahydrate and the solution was stirred. After stirring the solution was placed in an Amicon ultrafiltration unit containing a PM 10 ultrafiltration membrane designed to pass materials having a molecular weight <10,000 g/mol. The solution was diluted to 200 mL and then concentrated to 20 mL in volume. Inductively coupled plasma-atomic emission spectroscopy showed that the final solution had 18.5 mg/mL of Zn and 6.9 mg/mL of Cd.

## EXAMPLE U

A solution including gallium-doped zinc was prepared as follows. An amount of 200 mg of the concentrated solution from example N was mixed with 3.8 grams of the solution from example B. The resulting solution was clear and homogeneous. This method can be used to generate a wide variety of gallium doped zinc solutions by simply mixing in the appropriate ratios.

## EXAMPLE V

A solution including europium chloride and PEIC was prepared as follows. A europium solution with a carboxylated form of polyethylenimine (PEIC) was prepared by mixing 2.39 g of  $\text{EuCl}_3 \cdot 6\text{H}_2\text{O}$  with 1.52 g of the polymer. It was then filtered by the Amicon ultrafiltration unit containing a PM 10 ultrafiltration membrane with 200 mL of water and concentrated to 11.5 mL. The resulting solution of 13 wt % PEI and 0.49 wt % Eu was used for spin coating.

## EXAMPLE W

A solution including zirconyl nitrate and polyethylenimine was prepared as follows. An amount of 1.0 grams of

## 16

dipotassium ethylenediaminetetraacetic acid was dissolved in 30 mL of water. To this solution was added 2.0 grams of zirconyl nitrate (35 wt % in water) and the solution was stirred. Polyethylenimine (1 gram) was then added to the solution and the solution was stirred. The resulting solution is clear and has a pH of 8.0. This solution was placed in an Amicon ultrafiltration unit containing a PM 10 ultrafiltration membrane designed to pass materials having a molecular weight <10,000 g/mol. The solution was diluted to 200 mL with absolute ethanol and then concentrated to 10 mL in volume. Inductively coupled plasma-atomic emission spectroscopy showed that the final solution had 19.3 mg/mL of Sr.

## EXAMPLE X

A solution including titanium catecholate and polyethylenimine was prepared as follows. Titanium solutions were prepared using a titanium catecholate precursor. A solution of 2 g of PEI in 40 mL of deionized water was added to a mixture containing 2 g of  $\text{Ti}(\text{cat})_3(\text{NH}_4)_2$  dissolved in 20 mL of deionized water. This deep red solution was then heated for 20 minutes at 80°C. Upon cooling a precipitate was observed. The solution was stirred for a further 24 hrs at room temp then filtered through Celite. The deep red solution was filtered using an Amicon ultrafiltration unit containing a PM 10 ultrafiltration membrane, to give clean solution. Inductively coupled plasma-atomic emission spectroscopy showed that the final solution had 1.4 mg/mL of Ti.

## EXAMPLE Y

A solution including barium titanium catecholate and polyethylenimine was prepared as follows. An amount of 500 mg of  $\text{BaTi}(\text{cat})_3$  was dissolved in 40 mL of water. This was then added to a solution of PEIC (2 g PEIC dissolved in 40 mL of water). This deep red solution was stirred for 24 hrs and then all of the solvent was removed at reduced pressure. The resultant oil was re-dissolved in water (40 mL) and filtered through Celite™ diatomaceous earth to give a clear solution.

## EXAMPLE Z

A solution including yttrium, barium and copper was prepared as follows. Three equimolar solutions of yttrium nitrate (1.36 grams yttrium nitrate hexahydrate, 1.0 grams ethylenediaminetetraacetic acid, 1.2 grams polyethylenimine, 30 mL water), barium nitrate (0.90 grams barium nitrate, 1.0 grams ethylenediaminetetraacetic acid, 1.2 grams polyethylenimine, 30 mL water), and copper nitrate (0.85 grams copper nitrate trihydrate, 1.0 grams ethylenediaminetetraacetic acid, 1.2 grams polyethylenimine, 30 mL water) with ethylenediamine tetraacetic acid and polyethylenimine were prepared and then mixed in a 1:2:3 ration Y:Ba:Cu. The final solution was concentrated by rotary evaporation under reduced pressure.

## EXAMPLE AA

Metals can be directly bound by adding metal salts to the polymer solution. This has been demonstrated with PEI and Co, Ni, Pd, Zn and Cu as follows and with the PEIC polymer and Ti, Sn, Eu (as described above). A palladium chloride and polyethylenimine polymer solution was prepared by dissolving 1.0 grams of polyethylenimine in 40 mL of water and adjusting the pH to 6 with addition of 10% HCl. To this polymer solution was added 1.0 gram of palladium chloride and the solution was stirred. The solution pH was adjusted to

pH 1 to get complete dissolution and then titrated back to pH 6 with NaOH. After stirring, the solution filtered with a 0.45 micron filter and then placed in an Amicon filtration unit containing a PM 10 filter designed to pass materials having a molecular weight <10,000 g/mol. The retained solution was diluted to 200 mL and then concentrated to 20 mL in volume. Inductively coupled plasma-atomic emission spectroscopy showed that the final solution 425 mM Pd. Solutions of Co, Ni, Cu, and Zn bound to PEI were made in a similar manner although they did not require acidic conditions to dissolve. In these cases the metal salt was added to PEI and the pH was adjusted to near 7 with 10% HCl. The solutions were then purified by ultrafiltration through the Amicon filtration unit containing a PM 10 filter. A metal concentration greater than 10 mM indicates substantial binding to the polymer and the particular metal concentrations of these solutions are shown in Table 1. Final metal concentrations can be readily altered by adding water or concentrating by rotary evaporation.

TABLE 1

| Metal salt                                                  | Polymer   | Final [metal] |
|-------------------------------------------------------------|-----------|---------------|
| 1.0 g PdCl <sub>2</sub>                                     | 1.0 g PEI | 425 mM        |
| 0.85 g Cu(NO <sub>3</sub> ) <sub>2</sub> ·3H <sub>2</sub> O | 1.2 g PEI | 330 mM        |
| 1.0 g ZnCl <sub>2</sub>                                     | 1.0 g PEI | 350 mM        |
| 1.8 g CoCl <sub>2</sub>                                     | 1.8 g PEI | 181 mM        |
| 2.0 g NiCl <sub>2</sub>                                     | 2.0 g PEI | 441 mM        |

## EXAMPLE BB

Metal oxide clusters can be bound as anions to the polymer. This has been demonstrated with PEI and Si, W, and V. A silicon and polyethylenimine polymer solution was prepared by dissolving 7.0 grams of polyethylenimine in 70 mL of water followed by the addition of 8 g of water glass (50/50 wt % solution of Na and Si containing negatively charged silicate oligomers). The solution was titrated to pH 6 using 10% HCl. After stirring the solution (at pH 6) filtered through Celite<sup>TM</sup> diatomaceous earth and then placed in an Amicon filtration unit containing a PM 10 filter designed to pass materials having a molecular weight <10,000 g/mol. The solution was diluted to 200 mL and then concentrated to 80 mL in volume. This process was repeated three times to remove the unwanted sodium. Inductively coupled plasma-atomic emission spectroscopy showed that the final was 473 mM in Si. Vanadium and tungsten were bound as metal oxide clusters in a similar manner except that the metal oxide clusters are only stable at acidic pH. Solutions of the metal oxide clusters at pH 4 were added to PEI in solution at pH 4 and stirred. The pH can then be adjusted to 6 followed by purification by Amicon filtration. Alternatively the solution can be purified directly by ultrafiltration with no pH adjustment. The particular metal concentrations of these solutions are shown in Table 2.

TABLE 2

| Metal complex                      | Polymer           | Final [metal] |
|------------------------------------|-------------------|---------------|
| 1.9 g sodium orthovanadate at pH 4 | 2.0 g PEI at pH 4 | 139 mM        |
| 1.5 g sodium tungstate at pH 4     | 1.5 g PEI at pH 4 | 257 mM        |
| 8 g water glass (50/50 wt % Si/Na) | 7 g PEI           | 473 mM        |

## EXAMPLE CC

Metals can be bound to PEI as fluoride complexes as follows. Gallium nitrate (1.0 g) was dissolved in 20 mL of water followed by the addition of 0.67 g of ammonium bifluoride to generate the GaF<sub>6</sub><sup>3-</sup> anion. PEI (1.0 g) was then added and the mixture was purified by ultrafiltration.

## EXAMPLE DD

Metals can also be bound to PEI as EDTA complexes of the metals. This has been demonstrated with zinc (Zn), hafnium (Hf), gallium (Ga), neodymium (Nd), yttrium (Y), barium (Ba), strontium (Sr), bismuth (Bi), manganese (Mn), cerium (Ce), indium (In), europium (Eu), lanthanum (La), aluminum (Al), calcium (Ca), and lead (Pb). For a solution of zinc chloride, dipotassium ethylenediaminetetraacetic acid and polyethylenimine, 2.0 grams of dipotassium ethylenediaminetetraacetic acid were dissolved in 30 mL of water. Then, 0.75 grams of zinc chloride were added and the solution was stirred. After stirring, 2 grams of polyethylenimine were added. The solution was placed in an Amicon filtration unit containing a PM 10 filter designed to pass materials having a molecular weight <10,000 g/mol. The solution was diluted to 200 mL and then concentrated to 20 mL in volume. Inductively coupled plasma-atomic emission spectroscopy showed that the final solution was 373 mM Zn. The other metals including Hf, Ga, Nd, Y, Ba, Sr, Bu, Mn, Ce, In, Eu, La, Al, Ca, and Pb were each bound to PEI as EDTA complexes of the metals in a similar manner. The particular metal concentrations of these solutions are shown in Table 3.

TABLE 3

| Metal Salt                                                    | Polymer           | EDTA  | Final [metal] |
|---------------------------------------------------------------|-------------------|-------|---------------|
| 1.0 g HfOCl <sub>2</sub>                                      | 1.0 g PEI         | 1.0 g | 155 mM        |
| 1.0 g Ga(NO <sub>3</sub> ) <sub>3</sub>                       | 1.0 g PEI         | 1.0 g | 230 mM        |
| 1.5 g PbCl <sub>2</sub>                                       | 1.5 g PEI         | 1.5 g | 234 mM        |
| 3.0 g La(NO <sub>3</sub> ) <sub>3</sub>                       | 2.0 g PEI         | 2.0 g | 172 mM        |
| 1.3 Y(NO <sub>3</sub> ) <sub>3</sub> ·6H <sub>2</sub> O       | 1.0 g PEI         | 1.0 g | 115 mM        |
| 40 1.5 g Nd(NO <sub>3</sub> ) <sub>3</sub> ·6H <sub>2</sub> O | 1.0 g PEI         | 1.0 g | 158 mM        |
| 1.5 g CeCl <sub>3</sub> ·7H <sub>2</sub> O                    | 1.2 g PEI at pH 4 | 1.2 g | 134 mM        |
| 1.0 g EuCl <sub>3</sub>                                       | 1.0 g PEI         | 1.0 g | 136 mM        |
| 0.5 g Ca(OH) <sub>2</sub>                                     | 4.0 g PEI         | 4.0 g | 152 mM        |
| 45 1.7 g MnCl <sub>2</sub> hydrate                            | 1.8 g PEI         | 1.7 g | 216 mM        |
| 1.7 g Al <sub>2</sub> (SO <sub>4</sub> ) <sub>3</sub> hydrate | 1.9 g PEI         | 1.7 g | 182 mM        |
| 2.0 g Al(NO <sub>3</sub> ) <sub>3</sub> hydrate               | 2.0 g PEI         | 2.0 g | 245 mM        |
| 1.0 g Bi(NO <sub>3</sub> ) <sub>3</sub>                       | 1.0 g PEI         | 1.0 g | 101 mM        |

## EXAMPLE 1

The europium metal containing solution from Example V was used to spin coat films onto substrates of lanthanum aluminum oxide (LaAlO<sub>3</sub>). Spin coating was readily achieved with a spinning speed of 1500 rpm over 30 seconds. 55 (Spin Coater Model 100, from Cost Effective Equipment, a division of Brewer Science, Inc., Rolla, Mo.)

The resultant coating of polyethylenimine and europium metal was gradually heated from room temperature to about 1000-1200° C. over a period of about one hour under an oxygen atmosphere. FIG. 1 shows the general temperature profile of the thermal treatment for epitaxial growth of films deposited by the process of this invention. This heating process yielded polymer-free metal oxide films on the LaAlO<sub>3</sub> substrates. An x-ray diffraction 2θ-scan of the resultant europium oxide (Eu<sub>2</sub>O<sub>3</sub>) film is shown in FIG. 2. The film was preferentially oriented out of the plane. FIG. 3 shows the □-scans of (440) Eu<sub>2</sub>O<sub>3</sub> and (101) LaAlO<sub>3</sub>. The film is also

19

oriented in the plane. The epitaxial nature of the film deposited using this invention is further evidenced by the transmission electron microscopy as shown in FIG. 4 (high-resolution transmission electron microscopy) and FIG. 5 (selected electron diffraction pattern of a  $\text{Eu}_2\text{O}_3$  film on the  $\text{LaAlO}_3$  substrate). The interface between the substrate and the  $\text{Eu}_2\text{O}_3$  film is very sharp. No voids and second phases were detected in the film.

## EXAMPLE 2

The titanium metal containing solution from Example I was used to spin coat films onto R-cut sapphire substrates. Spin coating was readily achieved with a spinning speed of 1500 rpm over 30 seconds.

The resultant coating of polyethyleneimine and titanium metal was gradually heated from room temperature to about 1100-1200° C. over a period of about one hour under an oxygen atmosphere. This heating process yielded polymer-free metal oxide films on the sapphire substrates. The x-ray diffraction 20-scan of the titanium oxide ( $\text{TiO}_2$ ) film on the R-cut sapphire substrate is shown in FIG. 6. The film has a rutile structure and was preferentially oriented out of the plane. The epitaxial nature of the rutile  $\text{TiO}_2$  on R-cut sapphire is further evidenced by the high-resolution transmission electron microscopy and selected electron diffraction pattern (not shown over here). The interface between the substrate and the  $\text{TiO}_2$  film is very sharp. No voids and second phases were detected in the film.

## EXAMPLE 3

The titanium metal containing solution from Example I was used to spin coat films onto  $\text{LaAlO}_3$  substrates. Spin coating was readily achieved with a spinning speed of 1500 rpm over 30 seconds.

The resultant coating of polyethyleneimine and titanium metal was gradually heated from room temperature to about 980° C. over a period of about one hour under an oxygen atmosphere. This heating process yielded polymer-free metal oxide films on the sapphire substrates. The x-ray diffraction 20-scan of the titanium oxide ( $\text{TiO}_2$ ) film on the  $\text{LaAlO}_3$  substrate is shown in FIG. 7. The film has an anatase structure and was preferentially oriented out of the plane. The epitaxial nature of the anatase  $\text{TiO}_2$  on  $\text{LaAlO}_3$  is further evidenced by the  $\square$ -scans of (101)  $\text{TiO}_2$  and (101)  $\text{LaAlO}_3$  as shown in FIG. 8.

## EXAMPLE 4

The zinc metal containing solutions from Example A, B or C were used to spin coat films onto c-cut sapphire substrates. Spin coating was readily achieved with a spinning speed of 1500 rpm over 30 seconds.

The resultant coatings of polyethyleneimine and zinc metal were gradually heated from room temperature to about 750-1200° C. over a period of about one hour under an oxygen atmosphere. This heating process yielded polymer-free metal oxide films on the sapphire substrates. The epitaxial nature of the zinc oxide on c-cut sapphire was evidenced by the high-resolution transmission electron microscopy and selected electron diffraction pattern (not shown over here). The interface between the substrate and the zinc oxide film is very sharp. No voids and second phases were detected in the film.

It should be noted that no significant difference (in terms of the structure) was found between the solutions prepared from

20

example A, B or C. However, the zinc oxide film has better surface morphology as detected from the optical scope where solution C was used.

## EXAMPLE 5

The yttrium, barium and copper metal containing solution from Example Z was used to spin coat films onto  $\text{LaAlO}_3$  substrates. Spin coating was readily achieved with a spinning speed of 1500 rpm over 30 seconds.

The resultant coating of polyethyleneimine and yttrium, barium and copper metal was gradually heated from room temperature to about 800-980° C. over a period of about one hour under an oxygen atmosphere. This heating process yielded polymer-free metal oxide films of YBCO on the substrates. The x-ray diffraction 20-scan of the YBCO film on the  $\text{LaAlO}_3$  substrate is shown in FIG. 9. The film is highly c-axis oriented and shows no detectable second phase. The epitaxy nature of the YBCO on  $\text{LaAlO}_3$  is further evidenced by the  $\phi$ -scans of (102) YBCO and (101)  $\text{LaAlO}_3$  as shown in FIG. 10.

## EXAMPLE 6

The barium and titanium metal containing solution from Example P was used to spin coat films onto  $\text{LaAlO}_3$  substrates. Spin coating was readily achieved with a spinning speed of 1500 rpm over 30 seconds.

The resultant coating of related polymer and barium and titanium metal was gradually heated from room temperature to about 1200° C. over a period of about one hour under an oxygen atmosphere. This heating process yielded polymer-free metal oxide films of  $\text{BaTiO}_3$  on the substrates. The x-ray diffraction 20-scan of the  $\text{BaTiO}_3$  film on the  $\text{LaAlO}_3$  substrate is shown in FIG. 11. The film is highly oriented out of the plane and shows no detectable second phase. The epitaxy nature of the  $\text{BaTiO}_3$  on  $\text{LaAlO}_3$  is further evidenced by the  $\phi$ -scans of (101)  $\text{BaTiO}_3$  and (101)  $\text{LaAlO}_3$  as shown in FIG. 12.

## EXAMPLE 7

The strontium and titanium metal containing solution from Example Q was used to spin coat films onto  $\text{LaAlO}_3$  substrates. Spin coating was readily achieved with a spinning speed of 1500 rpm over 30 seconds.

The resultant coating of related polymer and strontium and titanium metal was gradually heated from room temperature to about 1200° C. over a period of about one hour under an oxygen atmosphere. This heating process yielded polymer-free metal oxide films of  $\text{SrTiO}_3$  on the substrates. The x-ray diffraction 20-scan of the  $\text{SrTiO}_3$  film on the  $\text{LaAlO}_3$  substrate is shown in FIG. 13. The film is highly oriented out of the plane and shows no detectable second phase. The epitaxial nature of the  $\text{SrTiO}_3$  on  $\text{LaAlO}_3$  is further evidenced by the  $\phi$ -scans of (202)  $\text{SrTiO}_3$  and (202)  $\text{LaAlO}_3$  as shown in FIG. 14.

## EXAMPLE 8

An amorphous glass substrate was coated with a conducting film of indium tin oxide. A glass slide was dipped into the solution from example O. The solution coated half of the glass slide. The glass slide was then placed into a furnace and gradually heated at 10° C./minute up to 300° C., held at 300° C. for 1 hour, heated at 10° C./minute to 400° C., held at 400° C. for 30 minutes and then allowed to cool. Resistance mea-

21

surements showed that the uncoated glass was non-conductive (resistance>Mohms), and the coated half had resistances as low as 20,000 Ohms.

## EXAMPLE 9

A porous Anodisc membrane (aluminum oxide) was coated with zinc oxide to make the membrane more stable in a corrosive environment. An Anodisc membrane with 200 nm pores was wetted with a drop of solution from example W. The membrane was allowed to dry for two hours. The membrane was then placed into a furnace and gradually heated at 10° C./minute to 300° C., held at 300° C. for 1 hour, heated at 10° C./minute to 400° C., held at 400° C. for 30 minutes, heated at 10° C./minute to 500° C., held at 500° C. for 1 hour and then allowed to cool. Corrosion tests with concentrated hydrochloric acid showed that the zirconium oxide coated membrane was able to withstand 5 hours of concentrated hydrochloric acid with no adverse effects. An uncoated membrane breaks apart and dissolves turning the solution yellow in the same period of time. The solution with the zirconium coating showed no yellowing and the membrane retained its porosity as evidenced by the transparency when wet.

The results of these examples for films of europium oxide, zinc oxide, titanium dioxide, and mixed complex oxides such as BaTiO<sub>3</sub>, SrTiO<sub>3</sub>, and YBa<sub>2</sub>Cu<sub>3</sub>O<sub>7-X</sub> demonstrate that epitaxial films can be achieved using the process or technique of the present invention. This technique could therefore provide a cost effective and easy route to such complex metal oxides as YBCO used in the superconducting field as well as a wide range of applications in other areas such as doped zinc oxide and indium tin oxide films for transparent conductors, zirconium oxide as a hardening/anticorrosion layer, Eu<sub>2</sub>O<sub>3</sub> as a buffer layer or as a dielectric materials, BaTiO<sub>3</sub> and SrTiO<sub>3</sub> as dielectric layer for capacitors and microwave devices. The use of metal oxides is extensive. Epitaxial growth means that the technique could be used for demanding electronic applications. The low decomposition temperature of PEI and PEIC makes such polymers desirable for glass coatings for optics/electrooptics applications. As these films can be made readily by spin coating or dip coating means that a wide variety of material types and shapes can be readily used. This may extend the range of applications to include metal oxide catalysts for catalytic converters and protective coatings for metal-based membranes.

## EXAMPLE 10

A palladium metal film was prepared as follows by spin coating a surface with the polymer and metal solution followed by removal of the polymer under a 5% hydrogen atmosphere. A palladium solution prepared as described in example AA was spin coated onto a glass slide at 2000 rpm. The slide was then heated in a 5% hydrogen atmosphere at 1° C./min to 120° C. with a dwell time of 30 min followed by heating to 350° C. at 1° C./minute with a dwell time of 30 min followed by heating to 450° C. at 1° C./minute with a dwell time of 1 hour and then cooling to 25° C. The resulting film was shown to be a continuous palladium film by XRD analysis and conductivity.

## EXAMPLE 11

A zirconium phosphate film was prepared by adding a stoichiometric amount of phosphate in the form of phosphoric acid to a solution of zirconium bound to PEI. The solution was then spin coated onto a glass slide and thermally treated

22

at 1° C. to 120° C. with a dwell time of 30 minutes followed by heating to 350° C. at 1° C./minute with a dwell time of 30 minutes followed by heating to 450° C. at 1° C./minute with a dwell time of 1 hour and then cooling to 25° C.

5

## EXAMPLE 12

An epitaxial film of strontium titanate with amorphous silicon nanoparticles was prepared as follows. A solution of silica particles was prepared by mixing 4g of PEI with 2.5 g of Ludox AS-30 to yield a homogeneous solution. This solution was then combined with a solution of Ti bound to PEIC and a solution of strontium bound to PEI to yield a solution with a metal ratio of Ti:Sr:Si of 1:1:0.3. This solution was spin coated onto a crystal of lanthanum aluminum oxide and thermally treated to yield an epitaxial film with amorphous silicon particle as evidenced by TEM and XRD.

20

## EXAMPLE 13

Porous epitaxial films of strontium titanate were prepared by heating the spin coated lanthanum aluminum oxide to 110° C. at a rate of 1° C./minute with a dwell time of 60 minutes followed by heating to 300° C. at 1° C./minute with a dwell time of 30 minutes followed by heating to 500° C. at 1° C./minute with a dwell time of 60 min followed by heating to 800° C. at 20° C./minute with a dwell time of 60 minutes and then cooling to room temperature at 20° C./minute.

30

## EXAMPLE 14

A polymer solution was coated onto and into a porous substrate as follows. Alumina anodiscs with 200 nm pores were coated with titanium dioxide using a solution of Ti bound to PEIC and with zirconium oxide using a solution of zirconium bound to PEI. The optimal metal concentration in the solution was between 100 and 300 mM. The solution was allowed to fill the pores and the alumina supports were then thermally treated at 1° C. to 120° C. with a dwell time of 30 minutes followed by heating to 350° C. at 1° C./minute with a dwell time of 30 min followed by heating to 500° C. at 1° C./minute with a dwell time of 1 hour and then cooling to 25° C. XRF analysis shows a uniform coating on the alumina disc and none of the pores are blocked.

45

## EXAMPLE 15

Gallium nitride is prepared with a solvent of water or ethanol using GaF<sub>6</sub><sup>3-</sup> bound to the PEI. The solution from example CC is readily spin coated and is then thermally treated in an ammonia atmosphere to generate the gallium nitride film.

55

## EXAMPLE 16

Zinc Telluride is prepared with a solvent of water or ethanol using Zn<sup>2+</sup> bound to the PEI, with an equivalent of bis(thiourea)tellurium dichloride added. The solution from example A is mixed with the equivalent of bis(thiourea)tellurium dichloride and is readily spin coated. Thereafter, it is then thermally treated in an argon atmosphere to generate the zinc telluride film.

60

Although the present invention has been described with reference to specific details, it is not intended that such details should be regarded as limitations upon the scope of the invention, except as and to the extent that they are included in the accompanying claims.

What is claimed is:

1. A process of preparing a uniform highly ordered metal oxide film comprising:
  - preparing a homogeneous solution comprising a suitable solvent, a soluble metal precursor, and a soluble polymer selected from the group consisting of polyethyleneimine, carboxylated polyethyleneimine, other PEI derivatives, polyacrylic acid, polypyrrolidone, and poly(ethylene-maleic acid), the homogeneous solution having a pH in a range of from about 4 to about 9;
  - purifying and concentrating the homogeneous solution by diluting it and thereafter passing a resulting diluted homogeneous solution through an ultrafiltration membrane, whereby impurities pass through the ultrafiltration membrane in a filtrate and a purified and more concentrated homogeneous solution is retained by the ultrafiltration membrane;
  - coating a substrate with the purified and concentrated homogeneous solution, thereby forming a polymer and metal containing layer thereon; and
  - heating said substrate in an oxygen-containing atmosphere at temperatures and for time characterized as sufficient to remove said polymer from said polymer and metal containing layer and form a uniform highly ordered metal oxide film.
2. The process of claim 1 wherein said metal is selected from the group consisting of alkali metals, alkaline earth metals, main group metals, transition metals, and lanthanide metals.
3. The process of claim 1 wherein said metal is selected from the group consisting of main group metals, lanthanide metals and alkaline earth metals.
4. The process of claim 1 wherein said uniform highly ordered metal oxide film is characterized as nanocrystalline.
5. The process of claim 1 wherein said uniform highly ordered metal oxide film is characterized as epitaxial.
6. The process of claim 1 wherein said uniform highly ordered metal oxide film is characterized as polycrystalline.
7. The process of claim 5 wherein said uniform highly ordered metal oxide film further includes nanoparticles.
8. The process of claim 7 wherein said nanoparticles are of silica.
9. The process of claim 1 wherein said uniform highly ordered metal oxide film is further characterized as porous and said process includes heating said substrate in an oxygen-containing atmosphere at temperatures, rates and time characterized as sufficient to remove said polymer from said polymer and metal containing layer and form a porous metal oxide film.
10. The process of claim 2 wherein said uniform highly ordered metal oxide film includes at least two of said metals.
11. The process of claim 1 wherein said uniform highly ordered metal oxide film is epitaxial europium oxide and said substrate is selected from the group consisting of lanthanum aluminum oxide, strontium titanate and lanthanum strontium aluminum tantalate.
12. The process of claim 1 wherein said solvent is selected from the group consisting of water, lower alcohols, acetone, tetrahydrofuran, propylene carbonate, acetonitrile, ethylacetate, acetic acid, and mixtures thereof.

13. The process of claim 1 wherein said solvent is selected from the group consisting of water and lower alcohols.
14. The process of claim 12 wherein said solvent is water and is organic-solvent free.
15. The process of claim 12 wherein said solution further includes a metal-binding ligand or salts thereof.
16. The process of claim 15 wherein said metal-binding ligand is EDTA or salts thereof.
17. The process of claim 1 wherein said uniform highly ordered metal oxide film includes zinc oxide.
18. The process of claim 1 wherein said uniform highly ordered metal oxide film includes titanium oxide.
19. The process of claim 18 wherein said titanium oxide is of a rutile form.
20. The process of claim 1 wherein said uniform highly ordered metal oxide film includes zirconium oxide.
21. The process of claim 18 wherein said titanium oxide is of an anatase form.
22. The process of claim 1 wherein said uniform highly ordered metal oxide film is a yttrium barium copper oxide film.
23. The process of claim 14 wherein said uniform highly ordered metal oxide film is a yttrium barium copper oxide film.
24. The process of claim 22 wherein said yttrium barium copper oxide film is epitaxial and is a superconductor.
25. The process of claim 23 wherein said yttrium barium copper oxide film is epitaxial and is a superconductor.
26. The process of claim 1 said uniform highly ordered metal oxide film is barium titanium oxide.
27. The process of claim 1 said uniform highly ordered metal oxide film is strontium titanium oxide.
28. The process of claim 1 wherein said solution is applied by a process selected from the group consisting of spin coating, dipping, spraying and ink jetting onto said substrate.
29. The process of claim 1 wherein said metal oxide is hafnium oxide.
30. The process of claim 1 wherein said uniform highly ordered metal oxide film is a conformal coating upon said substrate.
31. A process of preparing a uniform highly ordered metal oxide film comprising:
  - applying an aqueous homogenous solution of metal-bound polymer, said solution having a pH in a range of from about 4 to about 9, said solution prepared by combining a soluble metal precursor and a soluble polymer selected from the group consisting of polyethyleneimine, carboxylated polyethyleneimine, other PEI derivatives, polyacrylic acid, and poly(ethylene-maleic acid) in a suitable solvent which results in said metal-bound polymer, onto a substrate to form a layer of said metal-bound polymer,
  - heating said substrate in an oxygen-containing atmosphere at temperatures and for time characterized as sufficient to remove said polymer from said layer of metal-bound polymer and form a uniform highly ordered metal oxide film.